

Patented Dec. 5, 1922.

1,437,792

# UNITED STATES PATENT OFFICE.

STEWART J. CARROLL, OF ROCHESTER, NEW YORK, ASSIGNOR TO EASTMAN KODAK COMPANY, OF ROCHESTER, NEW YORK, A CORPORATION OF NEW YORK.

## CELLULOSE-ETHER SOLVENT AND COMPOSITION.

No Drawing.

Application filed April 5, 1921. Serial No. 458,737.

*To all whom it may concern:*

Be it known that I, STEWART J. CARROLL, a citizen of the United States of America, residing at Rochester, in the county of Monroe and State of New York, have invented certain new and useful Improvements in Cellulose-Ether Solvents and Compositions, of which the following is a full, clear, and exact specification.

10 This invention relates to solvents for making strong solutions of cellulose ether and also relates to the cellulose ether compositions produced by the aid of such solvents. One object of my invention is to provide a 15 solvent which will dissolve such large proportions of cellulose ethers that thick or viscous flowable solutions may be obtained for use in plastic and film making arts. Another object of my invention is to provide a 20 cellulose ether solution which may be manufactured into strong, flexible transparent film on the machines and by the methods now in use.

In U. S. Patent No. 1,188,376, Lilienfeld, 25 June 20, 1916, there are disclosed a series of alkyl ethers of cellulose. Certain of these are practically insoluble in water, and my invention relates but is not limited to the ethers having that property. While the 30 ethers form thin solutions in ethyl alcohol and the like, it has been found that such single solvents by themselves dissolve in general only a small proportion of the ethers, so that it is not possible to make a desirably 35 thick flowable composition or dope which may, for example, be used in the manufacture of photographic film base by customary methods, or in the other plastic arts.

I have discovered that an adequately 40 strong and useful solvent may be prepared by mixing the lower monohydroxy aliphatic alcohols (which are not strong enough solvents by themselves) with monochlornaphthalene. The combination of ethyl alcohol 45 and chloroform with monochlornaphthalene has been previously described, but I have discovered that the chloroform, which is relatively the most expensive of the ingredients, can be omitted.

50 While the proportions of my compound solvents may be greatly varied, I prefer those in which the monochlornaphthalene and lower monohydroxy aliphatic alcohols are present in substantially equal proportions. Methyl alcohol, ethyl alcohol and iso-

propyl alcohol are typical examples of the liquids which may be mixed with the monochlornaphthalene. I may also vary considerably the amount of ether that is dissolved in the compound solvent. By way of example, I may dissolve 1 part by weight of water-insoluble ethyl cellulose in 5 parts of the solvent, obtaining a thick viscous flowable solution. Other substances which impart additional suppleness to the film may then be added to the dope, such, for instance, as triphenyl or tricresyl phosphate, camphor, etc.

The ingredients are of the ordinary commercial type and sufficiently purified for the process of film manufacture, so as to give a dope yielding films having the proper relative freedom from color. The viscous-flowable dope above described can be used in connection with the usual film-forming apparatus 75 without the necessity of expensive alterations in the latter. The homologues of monochlornaphthalene and its isomers act equivalently, including the monochloranthracenes, etc. By the term lower monohydroxy aliphatic alcohols, I include such alcohols containing less than 6 carbon atoms.

Having thus described my invention, what I claim as new and desire to secure by Letters Patent is:

1. A compound solvent for alkyl ethers of cellulose, consisting of a mixture of monochlornaphthalene and a lower monohydroxy aliphatic alcohol.

2. A compound solvent for alkyl ethers of cellulose, comprising approximately equal parts by weight of monochlornaphthalene and of a lower monohydroxy aliphatic alcohol.

3. A viscous flowable film-forming composition, comprising an alkyl ether of cellulose dissolved in a mixture consisting essentially of monochlornaphthalene and a lower monohydroxy aliphatic alcohol.

4. A viscous flowable film-forming composition, comprising an alkyl ether of cellulose dissolved in a compound solvent consisting essentially of substantially equal parts of monochlornaphthalene and a lower monohydroxy aliphatic alcohol.

5. A composition of matter, comprising water-insoluble ethyl cellulose dissolved in a compound solvent consisting essentially of monochlornaphthalene and ethyl alcohol.

6. A composition of matter, comprising

water-insoluble ethyl cellulose dissolved in a compound solvent containing approximately equal parts by weight of monochlornaphthalene and ethyl alcohol.

5 7. A composition of matter, comprising cellulose ether dissolved in a compound consisting of a chlor-nucleo substitution prod-

uct of the hydrocarbons  $C_{2n}H_{n+3}$  and their homologues, and a lower monohydroxy aliphatic alcohol.

10

Signed at Rochester, New York, this 26th day of March, 1921.

STEWART J. CARROLL.